

## UNITED STATES PATENT OFFICE

WILLIAM B. PRICE, OF WATERBURY, CONNECTICUT, ASSIGNOR TO SCOVILL MANUFACTURING COMPANY, OF WATERBURY, CONNECTICUT, A CORPORATION OF CONNECTICUT

## NON-FERROUS ALLOY

No Drawing.

Application filed June 4, 1930. Serial No. 459,261.

This invention relates to a non-ferrous alloy, and particularly to an alloy comprising copper, aluminum, nickel, and tin as the essential ingredients.

Alloys have been made heretofore consisting essentially of copper, zinc and tin and are in general use on account of their valuable properties.

Also alloys consisting essentially of brass with a limited amount of aluminum are in general use and are valuable for many purposes.

I have discovered that alloys consisting essentially of copper, aluminum, nickel and tin, the said ingredients being within the general ranges hereinafter specified, have new valuable characteristics not heretofore found in the non-ferrous alloys of copper heretofore employed.

An alloy made in accordance with the present invention is suitable for the same uses as the prior copper, zinc, tin alloys and has the great advantage over the said alloys that it is more resistant to oxidation at high temperatures.

An alloy made in accordance with the present invention is practically immune to season cracking, and is more readily worked at hot and cold temperatures.

A further advantage of an alloy embodying the present invention is that its tensile strength is greater than that of the corresponding copper, zinc, tin alloy and that in its soft state it has a greatly increased percentage of elongation.

Another important advantage of an alloy made in accordance with the present invention is its remarkable physical properties at elevated temperatures. For example, at 500° C. it had a tensile strength of 28,900 pounds per square inch, whereas the prior alloys of copper, zinc and tin at the same temperature had a tensile strength of only 6,900 pounds per square inch. At a temperature of 750° C. the alloy constituting the present invention had a tensile strength of 4,300 pounds per square inch, an elongation of 55% in two inches and a reduction in area of 43%. The prior alloys of copper, zinc and tin, at the same temperature had a tensile strength of only 1,600 pounds per square inch, an elongation of 23% in two inches and a reduction in area of 24%.

An alloy made in accordance with the present invention comprises as essential ingredients the following metals; in about the ranges stated;

Copper from 80 to 85 parts, aluminum from 1 to 2½ parts, nickel from 1 to 2½ parts, tin from 1 to 2½ parts. Where the percentages of the above metals in any given alloy do not constitute one hundred percent, the difference most advantageously is zinc, but, of course, in practice other impurities may be present without injury to the resultant product. In practice it is found that as high as about 16 percent of zinc may be present and is advantageous for some purposes. Also, because it cannot be avoided without too much expense in refining the constituent metals, there may be and usually are some lead and iron present.

The following is an example of an alloy constituting the preferred embodiment of the invention for use as condenser tubes.

|               | Per cent |
|---------------|----------|
| Copper-----   | 80       |
| Aluminum----- | 2        |
| Nickel-----   | 1        |
| Tin-----      | 1        |
| Zinc-----     | 16       |

In commercial practice an alloy made from commercial material proportioned to give the composition above stated, when analyzed gave the following composition:

|               | Per cent |
|---------------|----------|
| Copper-----   | 80.20    |
| Aluminum----- | 2.25     |
| Nickel-----   | 1.14     |
| Tin-----      | 1.18     |
| Zinc-----     | 15.20    |
| Lead-----     | 0.01     |
| Iron-----     | 0.02     |

This commercial alloy when cast in a slab about  $\frac{3}{4}$  inch thick had a hardness of 65 on the Brinell scale. It was rolled as cast to 0.158 inch thick, then annealed for one hour at 750° C. to relieve it of internal stresses. Its hardness was still 65 Brinell. Then it was rolled to .050 inch finish gage. In this con-

dition its tensile strength was 112,000 pounds per square inch and the percentage of elongation of 2 inch test pieces was 3½. Its hardness on the Vicker's machine was equivalent to 230 Brinell.

- 8 The great advantage of this material for condenser tubes is its resistance to corrosion in salt water, apparently due to the formation of a protective scale or surface film resistant to oxidation by air, resistance to air impingement attack, the absence of red stains after pickling, which is a general defect of prior copper alloys made for similar uses, and particularly the increased tensile strength.
- 10 15 What I claim is:

1. An alloy comprising essential amounts of copper, aluminum, nickel, zinc, and tin in proportions substantially within the following ranges:

|          | Per cent |
|----------|----------|
| Copper   | 80 to 85 |
| Aluminum | 1 to 2½  |
| Nickel   | 1 to 2½  |
| Tin      | 1 to 2½  |
| Zinc     | 7½ to 17 |

20 25 2. An alloy consisting of the following ingredients in proportions substantially as stated:

|          | Per cent |
|----------|----------|
| Copper   | 80       |
| Aluminum | 2        |
| Nickel   | 1        |
| Tin      | 1        |
| Zinc     | 16       |

30 In testimony whereof, I have hereunto set my hand.

WILLIAM B. PRICE.